

1

2,944,931

## SANITARY PAPER AND PROCESS OF MAKING THE SAME

Christen H. C. Yang, Camas, Wash., assignor to Crown Zellerbach Corporation, San Francisco, Calif., a corporation of Nevada

No Drawing. Filed Dec. 13, 1957, Ser. No. 707,450

10 Claims. (Cl. 162—179)

This invention relates to a process of making sanitary papers having improved softness and surface feel and to the papers so produced. More particularly, the invention pertains to a process of incorporating lanolin into fibrous cellulosic papermaking slurries to be used in the production of sanitary paper.

As is well known, sanitary papers are used for disposable sanitary purposes. These papers are absorbent, bulky and have a rough finish. They include such grades as facial tissue, toilet tissue, paper napkins, towels and the like.

Many attempts have been made in the past to improve softness and surface feel of such papers in order to satisfy use requirements. Such attempts include mechanical treatments of paper, such as embossing, calendering, etc., as well as incorporation into the paper of a variety of chemical agents, usually referred to as softeners, plasticizers or humectants by means of impregnation or saturation of paper. Examples of such agents are glycerine, sorbital, urea, invert sugars and the like. These materials have the ability of absorbing and holding water. Since water alone is a good lubricant or plasticizer of cellulosic fibers, papers containing such humectants are characterized by being able to hold moisture therein at low relative humidities and in this way they keep the paper soft through the action of water.

While improvement in softness of certain grades of paper, particularly glassine or grease-proof papers, has been realized by impregnation with the above mentioned agents, such agents are not entirely satisfactory for the treatment of sanitary papers since they do not produce a softening effect desired by the trade. Moreover, such agents are applied to the finished sheet of paper by spraying, coating or impregnation; such impregnation procedures for paper require special equipment and give a paper product in which the humectant is unevenly distributed therein.

Accordingly, the present invention has as a principal object an improved process of making sanitary paper by incorporating lanolin in form of an aqueous emulsion into an aqueous slurry of papermaking fibers in such a manner that many of the disadvantages enumerated above are avoided.

Another object of this invention is to provide a process for the incorporation of an aqueous emulsion of lanolin into an aqueous papermaking slurry in such a manner that the addition of lanolin emulsion does not interfere with the conventional method of making paper on standard papermaking equipment.

Still another object of this invention is to provide a sanitary paper characterized by excellent softness and surface feel.

Still further objects and advantages of the present invention will be obtained from the following description and the appended claims.

The process of this invention of making sanitary papers having improved softness and surface feel broadly comprises providing a mixture of an aqueous slurry of cel-

2

lulosic papermaking fibers and an aqueous emulsion of lanolin used in an amount sufficient to impart the desired improvement in softness of the resulting paper. Precautions are taken at this point to insure that a substantial proportion of the lanolin content in the emulsion will be retained by the fibers.

Accordingly, the invention is based on the discovery that it is possible to produce a sanitary paper characterized by a marked improvement in softness by incorporating lanolin into an aqueous system containing papermaking fibers under such conditions that small, discrete lanolin particles will be deposited or adsorbed on individual fibers and such fibers will retain their property of felting or forming into a paper web on conventional papermaking equipment. The resulting paper has lanolin particles uniformly distributed throughout in contrast with papers which have received a surface treatment to improve softness.

Aqueous emulsions of lanolin may be prepared in the presence of a suitable emulsifying or dispersing agent. Although it is preferred to employ a cationic emulsifier in the preparation of such emulsions, non-ionic or anionic emulsifiers may also be used in certain cases. When a non-ionic or anionic aqueous emulsion of lanolin is to be added to the fibrous slurry, it may be desirable to incorporate into the slurry a cation-active substance in order to enhance the adsorption or deposition of lanolin particles on the cellulosic fibers which are normally of anionic character and thus attain a still greater softening effect of the resulting paper.

In accordance with the preferred embodiment of this invention, a cationic aqueous emulsion of lanolin is prepared using a cationic emulsifier in conjunction with lanolin and water. The cationic emulsifiers which may be employed in preparing a suitable lanolin emulsion in water are quaternary ammonium salts or bases, long chain amine salts, tertiary sulfonium salts or bases, quaternary sulfonium salts or bases, and the like. These may be used either singly or in combination with each other or with other well-known cationic emulsifiers. The quaternary ammonium compounds are examples of especially satisfactory emulsifiers; exemplary of these is a quaternary ammonium salt containing two long straight hydrocarbon chains within the same molecule.

Similarly, a wide variety of non-ionic emulsifiers may be used. Such emulsifiers are, in general, derivatives of aliphatic alcohols containing at least one free hydroxy group, particularly aliphatic polyhydroxy substances or polyhydric alcohols incompletely esterified with higher molecular weight aliphatic acids, particularly fatty acids; such compounds include monostearin, stearic acid mono-ester of diethylene or triethylene glycol, polyoxyethylene sorbitan stearates, and the like.

Typical anionic emulsifiers comprise the soaps of aliphatic acids, alkyl aryl sulfonates, alkyl aryl polyether sulfonates, fatty alcohol sulfates, sulfonated aliphatic compounds, and the like.

A wide variety of papermaking fibers may be used in the process of this invention. Such fibers in form of aqueous slurries may be derived from softwoods, hardwoods or annual plants including bagasse, cereal straws and the like. These various fibrous materials may be produced by conventional chemical pulping procedures such as sulfite, kraft, soda, as well as by mechanical treatment to produce groundwood.

An aqueous emulsion of lanolin of the cationic type, which is the preferred type of lanolin emulsion according to the present invention, may be prepared by simply adding lanolin, preferably in the molten condition, to cold water together with a suitable cationic emulsifier. The mixture is then vigorously agitated in a suitable mixing

apparatus, such as a colloid mill or a homogenizer until a uniform emulsion is obtained.

In addition to the two essential ingredients of the aqueous emulsion, namely lanolin and a cationic emulsifier, two auxiliary ingredients may be incorporated therein, if desired.

First, an emulsion stabilizer may be added in order to enhance the shelf-life and stability characteristics of the emulsion. Such stabilizers include several types of non-ionic surfactants, cellulose derivatives, proteins, phosphatides, lecithin, and the like.

Secondly, a certain quantity of an oil may be incorporated into the mixture, primarily in order to improve the paper machine operation, for example, by extending the life of the creping blade on the Yankee drier. Suitable oils comprise mineral, vegetable or animal oils having a specific gravity at 60° F. in the range of 0.80-0.99. Examples of mineral oils are lubricating oils produced by distillation of crude oil and having constituents boiling from about 600° F. at atmospheric pressure; light oils having a Saybolt viscosity at 100° F. of less than 175 and heavy oils of viscosity higher than 175 are satisfactory. Examples of vegetable oils are soya bean, cottonseed, and the like; examples of animal oil are whale oil, wool oil, lard oil, etc.

The respective amounts of the various ingredients described hereinabove which may be used in the preparation of the lanolin emulsion are shown in the following Table I in which the figures are expressed in percent by weight.

Table I

|            | Broad Range | Preferred Range |
|------------|-------------|-----------------|
| Lanolin    | 1-90        | 15-80           |
| Emulsifier | 10-90       | 20-50           |
| Stabilizer | 0-40        | 5-15            |
| Oil        | 0-80        | 10-40           |

It will be understood that water is present in the emulsion in an amount sufficient to produce an emulsion having a desired solids concentration which may range broadly from 0.1 to 50% and preferably from 5 to 25% by weight.

The aqueous emulsion of lanolin may be added to the aqueous slurry of papermaking fibers at any point prior to the paper web formation. Thus it may be added at the beater, mixing chest, or paper machine headbox. A very convenient method of adding the emulsion to the pulp slurry is by pumping it continuously into the paper machine headbox where adequate mixing of the components occurs rapidly and the particles of lanolin are instantly deposited on or adsorbed by the cellulosic fibers.

It will be appreciated that the amount of lanolin emulsion added to the pulp slurry may vary depending upon the type of fibers employed in the manufacture of the sanitary paper as well as on the degree of softness desired for such a paper. Generally the amount of lanolin added to the pulp slurry should be sufficient to improve softness and surface feel of the resulting paper. Usually an amount of from 0.1 to 40 pounds of lanolin and preferably from 0.5 to 10 pounds of lanolin per ton of oven-dry pulp will produce satisfactory improvement in softness of the resulting paper.

Also, if desired, other materials conventionally used as pulp additives may be incorporated into the pulp mixture. Such materials may include wet-strength resins such as urea-formaldehyde, melamine formaldehyde, etc. with or without acidifying agent, such as alum, starches, gums, etc., conventionally used as strengthening agents, as well as dyes or colorants usually employed in the paper-making.

The pH of the fibrous slurry is not critical as the de-

position of lanolin particles takes place at any pH level between about 2 and 9. As a result, the choice of pH will depend primarily on such factors as the character of the pulp and the presence or absence of wet-strength resins and colorants.

The lanolin-treated aqueous pulp slurry is then run on the paper machine wire or cylinder and the resulting paper is passed through heated drying rolls in the usual manner. Other desirable properties may be obtained by creping and/or calendering the paper.

The herein described invention will be further illustrated by means of the following examples which are intended to be descriptive of the invention in preferred embodiments thereof, percentages or parts being expressed by weight unless otherwise specified.

*Example 1.*—An aqueous emulsion of lanolin was prepared by placing in a mixing vessel 50 parts of anhydrous lanolin (U.S.P. grade) together with 50 parts of a cationic emulsifier, a quaternary ammonium salt containing two straight hydrocarbon chains of 16-18 carbon atoms in length within the same molecule, and mixing the two ingredients while heating at 120° F. to melt the mixture. The molten mixture was poured slowly into a vessel equipped with an agitator and containing 900 parts of cold water and mixed vigorously for 10 minutes at which time a coarse emulsion having a temperature of about 70° F. was formed. The resulting emulsion, having a solids content of 10%, was transferred to a colloid mill and treated therein until a stable, fine emulsion of lanolin was obtained.

To an aqueous fibrous slurry of 1% consistency, suitable for the manufacture of toweling, prepared by beating bleached softwood kraft pulp to 550 cc. Canadian Standard Freeness, there was added sufficient of the resulting emulsion to incorporate 1% of lanolin based on oven-dry pulp, corresponding to 20 pounds of lanolin per ton of oven-dry pulp. The mixture was agitated and formed into handsheets having a basis weight of 30 pounds per ream in accordance with the standard TAPPI procedure. For comparison, control handsheets were also made from the same pulp without lanolin emulsion added thereto.

The resulting papers were tested for softness in the Handle-O-Meter, supplied by the Thwing Albert Instrument Co., Philadelphia, Pennsylvania. The following table indicates the values obtained on the untreated controls and the lanolin-treated papers. It will be noted that the lower the value the better is the softness of the paper.

|                          | Control Paper | Lanolin-treated Paper |
|--------------------------|---------------|-----------------------|
| Softness, grams/4 inches | 31            | 21                    |

Thus the addition of a cationic lanolin emulsion to pulp slurry increased the softness of the resulting paper by approximately 32%, as compared to untreated paper.

Moreover, the lanolin-treated paper had a markedly improved surface feel and slightly improved absorbency.

*Example 2.*—In a manner essentially similar to that described in Example 1, an aqueous, cationic emulsion of lanolin was prepared. In addition to the two essential ingredients of Example 1, a mineral oil, Nujol, characterized by specific gravity of 0.88/0.90 at 60° F. and Saybolt viscosity of 360/390 at 100° F., was employed. The ingredients were admixed in amounts sufficient to give a 10% aqueous emulsion (solids basis) containing 30% of lanolin, 50% of cationic emulsifier and 20% of oil.

The emulsion was incorporated into the same paper-making fiber slurry as described in Example 1 in an amount corresponding to 0.6% of lanolin based on oven-dry pulp, or 12 pounds of lanolin per ton of oven-dry pulp.

The softness tests carried out in the same manner as in Example 1 gave the following results:

|                               | Control Paper | Lanolin-treated Paper |
|-------------------------------|---------------|-----------------------|
| Softness, grams/4 inches..... | 31            | 22                    |

Hence, the softness of the lanolin-treated paper was increased by about 29% and its examination indicated a significant improvement in surface feel, as compared to the untreated control paper.

*Example 3.*—An aqueous, cationic lanolin emulsion was prepared as indicated in Example 1, except that a non-ionic stabilizer, namely polyoxyethylene sorbitan monostearate, having a specific gravity of 1.08 at 25° C. and viscosity of 300 centipoises at 40° C. was added thereto. The ingredients were employed in amounts sufficient to provide a 10% aqueous emulsion (solids basis) containing 50% lanolin, 40% of cationic emulsifier and 10% of stabilizer.

The emulsion was added to the same kraft pulp slurry as employed in Example 1 in amount sufficient to provide 1% of lanolin based on the oven-dry pulp, corresponding to 20 pounds of lanolin per ton of oven-dry pulp.

The results of softness tests performed as indicated hereinabove were as follows:

|                               | Control Paper | Lanolin-treated Paper |
|-------------------------------|---------------|-----------------------|
| Softness, grams/4 inches..... | 31            | 20                    |

The resulting lanolin-containing paper had an increased softness by about 36% and markedly improved surface feel, as compared to the untreated control paper.

*Example 4.*—A stable, cationic, aqueous emulsion of lanolin having 20% solids was prepared as indicated above using the ingredients employed in the preceding examples in their respective quantities as follows: lanolin 27%, cationic emulsifier 42%, stabilizer 17% and oil 19%.

The emulsion was added to an aqueous pulp slurry of 0.5% consistency, comprising as a fibrous furnish 60% of bleached softwood kraft, 20% of bleached hardwood kraft and 20% of softwood groundwood, in an amount sufficient to provide 0.1% of lanolin based on oven-dry pulp, corresponding to 2 pounds of lanolin per ton of oven-dry pulp. The pulp mixture was formed into a creped tissue grade of paper having 13.8 pounds/ream basis weight.

The results of softness tests performed on this paper were as follows:

|                                       | Control Paper | Lanolin-treated Paper |
|---------------------------------------|---------------|-----------------------|
| Softness, grams/inch $\times$ 10..... | 38            | 27                    |

Thus, the lanolin-containing tissue paper had an increased softness by about 29% and markedly improved surface feel, compared to the untreated control paper.

*Example 5.*—To the same pulp slurry as indicated in Example 4 there was added an aqueous cationic emulsion of lanolin containing the same constituents as in Example 4, but used in the following amounts: lanolin 33%, cationic emulsifier 33%, non-ionic stabilizer 17%, and oil 17%. The amount of the emulsion added was sufficient to give 0.07% of lanolin, oven-dry pulp basis (1.4 pound per ton of pulp).

The creped paper of 13.5 pounds/ream basis weight, formed from the above mixture, was tested for softness

together with the same paper untreated with the lanolin emulsion. The results were as follows:

|                                       | Control Paper | Lanolin-treated Paper |
|---------------------------------------|---------------|-----------------------|
| Softness, grams/inch $\times$ 10..... | 38            | 34                    |

The resulting lanolin-treated tissue had an increased softness by about 11% and improved surface feel, as compared to the untreated control.

*Example 6.*—Three stable aqueous emulsions of lanolin having 20% solids, namely, a cationic, an anionic and a non-ionic emulsion, were prepared in the manner described hereinabove. The emulsions, designated A, B and C, respectively, contained the following ingredients in their respective proportions: (A) lanolin 20%, cationic emulsifier (the same as employed in Example 1) 51%, stabilizer (the same as employed in Example 3) 7%, and mineral oil (the same as employed in Example 2) 22%; (B) lanolin 20%, anionic emulsifier, e.g., N-octadecyl tetrasodium N-(1,2-dicarboxyethyl sulfo-succinate) 30%, stabilizer e.g., polyoxyethylene sorbitan monolaurate, 27%, and the same mineral oil 23%; (C) lanolin 20%, emulsifier, e.g., a mixture of 51% of polyoxyethylene sorbitan monolaurate and 7% of sorbitan monolaurate, and the same mineral oil 22%.

Each of the above identified emulsions was added separately to an aqueous pulp slurry of 1% consistency, comprising as a fibrous furnish bleached softwood kraft, in amounts sufficient to provide 0.2% of lanolin based on oven-dry pulp, corresponding to 4 pounds of lanolin per ton of oven-dry pulp, followed by addition of paper-maker's alum solution in amount sufficient to reduce the pH of the mixture to 5.0. The pulp mixtures were then formed into toweling paper grades of about 30 pounds/ream basis weight.

Another series of paper sheets was also made using the same lanolin-containing pulp slurries, to which cationic melamine-formaldehyde wet-strength resin was added in an amount of 1% (solids basis) on oven-dry pulp. Paper of the same basis weight was formed in the same manner as set forth hereinabove.

The results of softness tests performed on the resulting papers and on papers containing no lanolin were as follows:

|                              | Control Paper | Lanolin-treated Paper (A) | Lanolin-treated Paper (B) | Lanolin-treated Paper (C) |
|------------------------------|---------------|---------------------------|---------------------------|---------------------------|
| Softness, grams/4 inches:    |               |                           |                           |                           |
| No wet strength resin.....   | 42            | 28                        | 38                        | 32                        |
| With wet-strength resin..... | 44            | 28                        | 32                        | 29                        |

The above data indicate that the three types of lanolin emulsions produced an improvement of softness in the resulting papers, as compared to the same paper containing no lanolin. It is to be noted that softness was further improved through addition of a cation-active substance, e.g., melamine-formaldehyde resin, to pulp slurries treated with either anionic lanolin emulsion (B) or non-ionic lanolin emulsion (C) in particular. It will be also observed, that although the treatment of the control paper with the wet-strength resin alone affected adversely its softness characteristics, such characteristics were improved significantly by incorporation to pulp of a lanolin emulsion.

*Example 7.*—An aqueous, cationic emulsion of lanolin having a 20% solids content and containing 21% of lanolin, 17% of cationic emulsifier, 8% of non-ionic stabilizer and 54% mineral oil (all the ingredients being the same as in the preceding examples) was added continuously at the paper machine headbox to an aqueous slurry of fibers having 0.3% consistency and comprising

50% bleached softwood sulfite, 20% bleached softwood kraft, 20% hardwood groundwood and 10% bleached hardwood kraft, at such a rate as to provide 0.4% of lanolin, oven-dry pulp basis, corresponding to 8 pounds of lanolin per ton of oven-dry pulp.

The resulting pulp mixture was converted into creped household toweling paper grade having a basis weight of 35.2 pounds per ream.

Another paper machine run was made to produce, as a control, the same grade of paper without adding the lanolin emulsion. The test results were as follows:

|                                    | Control<br>Paper | Lanolin-<br>treated<br>Paper |
|------------------------------------|------------------|------------------------------|
| Softness, grams/inch $\times 10$ : |                  |                              |
| MD <sup>1</sup>                    | 13               | 10                           |
| CMD <sup>2</sup>                   | 35               | 24                           |
| Total                              | 48               | 34                           |

<sup>1</sup> Machine direction.

<sup>2</sup> Cross-machine direction.

Thus the lanolin-treated toweling had an increased softness by about 29% and was characterized by a markedly improved surface feel, as compared to the untreated control. Moreover, the lanolin-containing pulp slurry ran well on the paper machine and produced toweling which had other desirable properties required by the trade, such as absorbency, caliper, tensile and stretch. In addition, the creping blade on the Yankee drier lasted twice as long during the manufacture of lanolin-treated paper than during the manufacture of the untreated control paper.

*Example 8.*—Two similar paper machine runs were made using the same lanolin emulsion, as indicated in Example 7, but making facial tissue grade having 10.4 pounds/ream basis weight. Prior to the addition of the lanolin emulsion, 1% of a urea formaldehyde wet-strength resin (dry fiber basis) and sufficient papermaking alum to adjust the pH of the pulp mixture to 5.5 were added to the slurry, which was composed of 50% bleached softwood sulfite and 50% bleached hardwood kraft.

The lanolin emulsion was added continuously at the headbox at such a rate as to incorporate into the pulp 0.5% lanolin (oven-dry pulp basis), corresponding to 10 pounds of lanolin per ton of oven-dry pulp.

The resulting pulp mixture was run on the paper machine, creped on the Yankee drier and passed through two calender nips.

For comparison, the same grade of paper was made under the same conditions but without adding the lanolin emulsion. The results of softness tests were as follows:

|                           | Control<br>Paper | Lanolin-<br>treated<br>Paper |
|---------------------------|------------------|------------------------------|
| Softness, grams/8 inches: |                  |                              |
| MD                        | 5                | 3                            |
| CMD                       | 18               | 8                            |
| Total                     | 23               | 11                           |

The lanolin-treated tissue paper had an increased softness by about 52% and significantly improved surface feel, as compared to the same paper containing no lanolin. In addition, other physical properties of the resulting paper product were entirely satisfactory for a commercial grade of tissue paper.

The following working examples illustrate other embodiments of the invention:

*Example 9.*—Lanolin 22%; cationic emulsifier (a long chain amine salt), hexadecylamine acetate 16%; stabilizer, polyoxyethylene sorbitan tristearate 10%; saturat-

ing oil 52%. This may be combined with a pulp slurry for papermaking at the rate of 0.1 pound of lanolin per ton of pulp (oven-dry weight basis).

*Example 10.*—Lanolin 80% and cationic emulsifier (the same as in Example 1) 20%. This may be combined with a pulp slurry for papermaking at the rate of 0.5 pound of lanolin per ton of pulp (oven-dry weight basis).

*Example 11.*—Lanolin 15% and cationic emulsifier (the same as in Example 1) 85%. This may be combined with a pulp slurry for papermaking at the rate of 35 pounds of lanolin per ton of pulp (oven-dry weight basis).

*Example 12.*—Lanolin 30%; cationic emulsifier (another quaternary ammonium salt), N-cetyl N-ethyl morpholinium ethosulfate 30%; stabilizer (the same as in Example 9) 20%; Nujol oil 20%. This may be combined with a pulp slurry for papermaking at the rate of 0.5 pound of lanolin per ton of pulp (oven-dry weight basis).

*Example 13.*—Lanolin 40%; anionic emulsifier (alkyl aryl polyether sulfonate), sodium salt of alkyl aryl polyether sulfonate 40%; stabilizer (the same as in Example 9) 10%; Nujol oil 10%. This may be combined with a pulp slurry for papermaking at the rate of 3 pounds of lanolin per ton of pulp (oven-dry weight basis).

*Example 14.*—Lanolin 75%; non-ionic emulsifier, sorbitan mono-oleate 25%. This may be combined with a pulp slurry for papermaking at the rate of 12 pounds of lanolin per ton of pulp (oven-dry weight basis).

*Example 15.*—Lanolin 50%; cationic emulsifier (the same as in Example 1) 40%; stabilizer, lecithin 10%. This may be combined with a pulp slurry for papermaking at the rate of 40 pounds of lanolin per ton of pulp (oven-dry weight basis).

*Example 16.*—Lanolin 50%; cationic emulsifier (the same as in Example 1) 40%; vegetable oil (cottonseed) 10%. This may be combined with a pulp slurry for papermaking at the rate of 10 pounds of lanolin per ton of pulp (oven-dry weight basis).

*Example 17.*—Lanolin 50%; cationic emulsifier (the same as in Example 1) 40%; animal oil (lard) 10%. This may be combined with a pulp slurry for papermaking at the rate of 10 pounds of lanolin per ton of pulp (oven-dry weight basis).

Accordingly, it is apparent that by the present invention I have provided an improved process for the manufacture of sanitary papers which process includes incorporation into an aqueous pulp slurry of an aqueous lanolin emulsion. Through interaction of a cationic emulsifier, the process results in a rapid, uniform and more complete deposition of discrete lanolin particles on the fibers which in turn results in the formation of paper products characterized by excellent softness, surface feel and other properties prerequisite for such paper grades, as tissue, toweling, napkin and the like.

I claim:

1. The process of improving the softness and surface feel of sanitary paper, which comprises adding to an aqueous slurry of papermaking fibers a stable, aqueous emulsion of 1-90% by weight of lanolin and 10-99% by weight of a cationic emulsifier selected from the group consisting of quaternary ammonium salts, quaternary ammonium bases, quaternary sulfonium salts, quaternary sulfonium bases, long chain amine salts and tertiary sulfonium bases, said slurry and said emulsion being at substantially room temperature, whereby a substantial proportion of lanolin particles and emulsifier contained in said emulsion is deposited onto said fibers while said fibers are suspended in water, and thereafter forming a paper web from the resulting slurry, the amount of lanolin and emulsifier deposited on the fibers being sufficient to improve the softness and surface feel of the resulting paper but being insufficient to permit said lanolin from being rubbed off on said paper.

2. Sanitary paper product produced in accordance with the process of claim 1.

3. The process of claim 1 wherein the amount of lanolin added to the slurry of papermaking fibers is from 0.1 to 40 pounds per ton of oven-dry pulp.

4. The process of claim 1 wherein the amount of lanolin added to the slurry of papermaking fibers is from 0.5 to 10 pounds per ton of oven-dry pulp.

5. The process of claim 1 wherein the emulsion is prepared by adding a molten mixture of the lanolin and of the emulsifier to cold water and vigorously agitating the resulting aqueous mixture until a finely divided emulsion is obtained.

6. The process of claim 1 wherein the emulsion comprises essentially 15-80% by weight of lanolin and 15 20-50% by weight of the emulsifier.

7. The process of claim 1 wherein the emulsion has a solids content of 0.1-50% by weight.

8. The process of claim 1 wherein the emulsion has a solids content of 5-25% by weight.

9. The process of claim 1 wherein the emulsifier is a quaternary ammonium compound.

10. The process of claim 1 wherein the emulsifier is a quaternary ammonium salt containing two long straight hydrocarbon chains within the same molecule.

**References Cited in the file of this patent**

**UNITED STATES PATENTS**

|           |               |                |
|-----------|---------------|----------------|
| 2,173,243 | Young         | Sept. 19, 1939 |
| 2,442,972 | Edelstein     | June 8, 1948   |
| 2,601,598 | Daniel        | June 24, 1952  |
| 2,637,662 | Russell       | May 5, 1953    |
| 2,832,357 | Powers        | Apr. 29, 1958  |
| 2,877,115 | Wemyss et al. | Mar. 10, 1959  |

UNITED STATES PATENT OFFICE  
CERTIFICATE OF CORRECTION

Patent No. 2,944,931

July 12, 1960

Christen H. C. Yang

It is hereby certified that error appears in the printed specification of the above numbered patent requiring correction and that the said Letters Patent should read as corrected below.

Column 3, line 45, for "boardly" read -- broadly --;  
column 8, line 75, for "on" read -- of --.

Signed and sealed this 13th day of December 1960.

(SEAL)

Attest:

KARL H. AXLINE  
Attesting Officer

ROBERT C. WATSON  
Commissioner of Patents